

1

3,492,172

METHOD FOR PRODUCING TITANIUM STRIP  
Adrian Burt Sauvageot, Toronto, and James M. Partridge,  
Steubenville, Ohio, assignors to Titanium Metals Corporation of America, New York, N.Y.

No Drawing. Filed Nov. 9, 1966, Ser. No. 592,995  
Int. Cl. C22f 1/18, 1/16

U.S. Cl. 148—11.5

25 Claims

## ABSTRACT OF THE DISCLOSURE

Method for producing strip having a substantially recrystallized microstructure from commercially pure titanium, alpha, stabilized alpha type titanium base alloys, and alpha stabilized alpha-beta type titanium base alloys comprising unidirectionally hot rolling a metal body from a temperature requiring a substantial amount of reduction in the alpha-beta field, heating said rolled metal at a temperature above the beta transus of said metal to transform the crystal structure of said metal to the beta phase and rapidly cooling said metal to a temperature below the beta phase to produce an acicular type microstructure in the metal followed by rolling and annealing said metal at temperatures below the beta transus.

This invention relates to a method for the manufacture of titanium and titanium alloy strip which is particularly characterized by freedom from the tendency to either rib or ridge, good ductility and minimum anisotropy of mechanical properties. More particularly, the method of our invention permits the production of equiaxed substantially completely recrystallized elongated strip which may be rolled to finish gauge or fabricated. Our method may be successfully applied to commercially pure titanium and to alpha and alpha-beta type titanium alloys containing alpha stabilizers.

Ribbing and ridging are indicated by longitudinal striations which occur in titanium metal which has been unidirectionally rolled at temperatures high in the alpha-beta field and which are oriented in the direction of rolling. Ribbing refers to the striations which develop during subsequent rolling of the strip to finish gauge, and ridging refers to the striations which develop during testing of rolled strip or during fabrication of products therefrom. Both of these effects are believed to be caused by crystallographic orientations imparted to the metal during the unidirectional rolling of bars and billets into a hot band. Anisotropy is also created in the metal by unidirectional rolling and is evidenced by a difference between the mechanical properties of the strip when measured parallel to the direction of rolling and when measured transversely of the direction of rolling.

Since ribbing and ridging in titanium and titanium base alloys are apparently created by unidirectional rolling of the metal in or through the two-phase alpha-beta field, they could be avoided by rolling at temperatures sufficiently low to avoid deformation in the alpha-beta field. Additionally, ribbing, ridging and anisotropy of mechanical properties may be eliminated by cross rolling the metal body at right angles to the original direction of rolling to an extent to obtain approximately the same degree of reduction as obtained during the original rolling. However, low temperature rolling is not practical with titanium alloys since sufficient reduction cannot be obtained and cross rolling is not practical for the commercial production of either titanium or titanium alloy strip.

Initial rolling at temperatures in the beta field or relatively high in the alpha-beta field is essential for the production of a hot band of alpha and alpha-beta type titanium alloys for subsequent rolling to finish strip since

2

reduction of a billet or bar to a hot band involves a substantial decrease in size. This reduction must be initiated at elevated temperatures since the alloys have a low specific heat and a consequent rapid temperature drop, and it is important that the metal be sufficiently plastic to permit rapid and easy deformation. Although an elevated temperature is essential for easy deformation, the temperature should not be so high as to cause excessive oxidation and scaling of the metal surface during deformation. Practical temperatures from the standpoint of ease of deformation and avoidance of excessive contamination of the metal surface are high in the alpha-beta field or low in the beta field; and substantial reduction at other temperatures is not practical.

Although cross rolling will eliminate ribbing and ridging and will substantially decrease directionality, cross rolling is limited to sheet products having a length not much greater than their width since the dimensions of the sheet must be such that it can pass crosswise through the rolling mill. Since cross rolling is of necessity limited to sheets having a length no greater than the roll width, it obviously cannot be applied to elongated hot bands having lengths of a hundred feet or more which are to be rolled into even longer strips.

Heat treatment of commercially pure titanium and alpha and alpha-beta type titanium alloys by annealing at a temperature near the beta transus of the metal prior to reduction to eliminate ribbing and ridging and to decrease anisotropy is disclosed in United States Patent No. 3,169,085. While the method disclosed in this patent will reduce the tendency toward ribbing and ridging and will reduce anisotropy, the resulting microstructure of commercially pure titanium and alpha and alpha-beta type alloys processed in accordance with the method is such that ductility is extremely poor; and, therefore, the metal cannot be further reduced or fabricated without catastrophic internal shear cracking of the metal. The extent of the shear cracking has been found to be dependent upon the annealing temperature and the rate of cooling from the annealing temperature. In order to produce a strip which will not have a tendency to rib or to ridge and which can be successfully rolled and fabricated, we have found it essential that the strip be annealed at a temperature above the beta transus of the metal and that the strip be rapidly cooled to a temperature below the beta transus. Treatment in this manner creates a substantially completely acicular type microstructure in the metal as opposed to the lamellar or to the Widmanstatten type structure which is created when the metal is cooled at a slower rate. Rapid cooling in accordance with our invention may be obtained by immersion, spraying or extremely fast air cooling; and the method of cooling will depend upon the specific material and the thickness of the strip being processed. Annealing at a temperature above the beta transus and rapid cooling to a temperature below the beta transus are termed a beta quench hereinafter.

Summarized briefly, our invention provides a method for producing strip of commercially pure titanium and alpha and alpha-beta type titanium alloys containing alpha stabilizers which is characterized by freedom from ribbing and ridging, minimum anisotropy of mechanical properties and good ductility. Strip produced according to our invention can be cold rolled to finish gauge and fabricated without failure due to internal shear cracking. Basically, our method comprises unidirectionally hot rolling the metal from a temperature in its beta field or high in its alpha-beta field; heating the rolled metal to a temperature above its beta transus and rapidly cooling to a temperature below the beta transus to create a substantially completely acicular microstructure and subsequently deforming and annealing the metal to substantially completely recrystallize the microstructure. The beta quench may be performed

on the hot band immediately after the unidirectional rolling, or it may be performed later in the process after the hot band has been reduced. After the beta quench, it is necessary that the metal be subjected to deformation and annealing in a manner and to an extent to effect substantially complete recrystallization of the microstructure in the metal. It is essential that the microstructure be substantially completely recrystallized for the metal to have sufficient ductility to permit subsequent cold rolling and fabrication without failing due to internal shear cracking. The term cold rolling as used herein encompasses rolling between about room temperature and about 300° F.

Metal which may be advantageously treated by the method of our invention is selected from the group consisting of commercially pure titanium, alpha type titanium alloys and alpha-beta type titanium alloys. The alloys must be alpha stabilized since beta stabilized alpha-beta alloys are susceptible to the formation of the brittle omega phase during rapid cooling from the beta field. Commercially pure titanium is available in various grades depending upon hardness, and the compositions of the grades differ principally in the content of the interstitials, oxygen, nitrogen and carbon. Generally speaking, commercially pure titanium has alpha type microstructure at room temperature and will convert to the beta crystal form at temperatures above its beta transus. Alpha type titanium alloys have an alpha microstructure at room temperature and contain alpha stabilizers of which aluminum, tin and columbium are examples. An alloy containing 5% aluminum, 2.5% tin, balance titanium, is typical of the alpha type alloys. The alpha-beta type titanium alloys have a mixture of alpha type microstructure and beta type microstructure at room temperature and are exemplified by an alloy containing 6% aluminum, 4% vanadium, balance titanium. A group of alloys generally designated alpha lean beta type contain a substantial amount of alpha stabilizing agent and a minor proportion of beta stabilizing agent and are subject to treatment by our method since the alpha stabilizers predominate. An alloy containing 8% aluminum, 1% vanadium, 1% molybdenum, balance titanium is a typical alpha lean beta type.

The initial hot rolling step to reduce the bar, billet or other shape to hot band is initiated at a temperature in the beta field or high in the alpha-beta field of the metal being processed. Any type of rolling mill may be employed, and the dimensions of the starting shape are not material so long as the shape will fit into the mill. Conveniently, the initial rolling is carried out by heating the metal body to the starting temperature heat or above the beta transus and then passing it through the rolling mill, rolling being continued as the temperature of the metal drops. A large portion of the reduction and certainly the later part thereof is accomplished in the alpha-beta field of the metal being rolled due to the low specific heat of titanium and titanium base alloys.

After rolling, the metal is heated to a temperature above its beta transus. This is accomplished in any suitable manner by conventional apparatus and may be carried out by placing a coil in a furnace although it is preferable to continuously heat successive portions of a hot band or strip. Maintenance of titanium and titanium base alloys at a temperature above the beta transus for an extended period of time is undesirable because it coarsens the grain structure; and, if the heating is carried out without the protection of an inert atmosphere, surface oxidation and scaling occur. It is, however, essential that the metal be held above the beta transus for a sufficient time to insure complete transformation of the entire metal body to beta structure; and, therefore, the duration of the anneal will depend upon the temperature of the heating furnace and the size and shape of the body being heated. For example, in the case of a closely wound coil, sufficient time must be allowed for the innermost convolutions to be

raised to temperature. When a continuous anneal is utilized to raise successive portions of hot band or strip to temperature the time required at temperature will be very short since the hot band or strip will be rapidly heated throughout. The precise temperature employed for the anneal is not critical providing it is above the beta transus of the metal being treated. A preferred maximum is about 150° F. above the beta transus since this provides a margin of safety insuring complete heating above the beta transus and is not so high as to coarsen the grain size and produce excessive surface oxidation and scaling.

After the metal has been completely transformed to beta structure, it is rapidly cooled to produce the required substantially completely acicular microstructure for subsequent recrystallization. Rapid cooling of the metal to a temperature below the beta transus is absolutely essential for the success of our process as it is not possible to obtain recrystallization by subsequent deformation and annealing unless the metal is beta quenched to create the acicular microstructure necessary for recrystallization. As will be shown hereinafter, the ductility of unrecrystallized strip as determined by bend tests is low. Cooling may be accomplished by either immersion or spraying, and any coolant which will rapidly decrease the temperature of the metal may be used. Additionally, air cooling is sufficient to rapidly lower the temperature of very thin strip. As stated heretofore, the beta quench may be performed immediately after hot rolling, or it may be carried out as an intermediate step between reductions.

The precise temperature at which the microstructure will become substantially completely acicular in the rapidly cooled or beta quenched metal will vary depending largely on the particular composition of the metal, as will be appreciated by those skilled in the art. However, in all instances, this temperature will be lower than the beta transus of the metal. For practical application of the method, it is preferable to cool the heated metal to room temperature since the formation of the necessary acicular microstructure is insured and a minimum of control is required. However, it is not essential that the metal be cooled to room temperature; and if control conditions permit, it may be cooled to a temperature above room temperature.

In addition to cooling the metal to a temperature below its beta transus, it is necessary that the rate of cooling be rapid to produce acicular microstructure in the metal. This microstructure will be readily recognized by those skilled in the art by the appearance of a section of the metal cut, polished and etched by conventional techniques and examined under a microscope. The microstructure consists principally of needle-like grains more or less randomly oriented. The aciculas may have more than three habit planes, that is, they may be oriented or grouped in more than three directions. Such a microstructure is readily distinguishable from that obtained by slower cooling from the beta field which will consist principally of platelet alpha titanium in basketweave or Widmanstatten array. Usually the platelets will lie in no more than three directions in blocks smaller than the original beta grains. The acicular microstructure, formed by the rapid cooling from the beta field according to our invention, is readily broken up and recrystallized by subsequent deformation and annealing; and this substantially completely recrystallized microstructure provides good ductility in the final strip.

After the beta quench, the metal is treated by a sequence of rolling and annealing steps designed to create recrystallized microstructure in the metal. The deformation of the metal during rolling imparts strain to the metal, and subsequent annealing tends to relieve the strain and recrystallizes the grain structure. Partial stress relief is obtained by intermediate anneals, and the final anneal results in complete stress relief and substantially complete recrystallization. As would be expected, the precise sequence of rolling and annealing applied to the beta quenched metal and the temperature of these steps will

vary with the material and thickness being treated, the desired finish gauge of the strip and the equipment available. For certain materials a stress relief anneal is beneficial prior to any deformation immediately after the beta quench. Generally speaking, smaller reductions and longer intermediate anneals must be used with lower rolling temperatures to prevent internal shear cracking while larger reductions are required at higher rolling temperatures to impart the required strain to the metal for subsequent recrystallization.

It is possible to roll some titanium strip products, such as commercially pure titanium and an alloy containing 5% aluminum, 2.5% tin, balance titanium, at temperatures which permit recrystallization simultaneous with rolling. The rolling temperature for simultaneous recrystallization will be between about 1000° F. and 1200° F. for beta quenched commercial pure titanium and between about 1200° F. and 1400° F. for the alloy containing 5% aluminum, 2.5% tin, balance titanium. When recrystallization occurs during rolling, the final anneal will result in stress relief and grain growth and the resulting microstructure, which is substantially completely recrystallized, is large grained and less equiaxed than metal which is recrystallized by a final anneal only. Due to the grain size and orientation in metal which has partially recrystallized during rolling, the metal is less susceptible to further cold rolling than metal which is recrystallized by a final anneal. However, if no further reduction of the strip is required, rolling at temperatures which permit recrystallization is satisfactory as the strip produced has no tendency to rib or ridge, has low anisotropy and high ductility. For this reason, rolling temperatures for commercially pure titanium and the titanium alloy containing 5% aluminum and 2.5% tin should be based in part on the work to be done on the material after the rolling recrystallization cycle.

It is necessary that the rolling and annealing temperatures be kept below the beta transus of the metal since reheating to above the beta transus will require subsequent rapid cooling followed by rolling annealing to obtain the recrystallized structure. It has been found that temperatures ranging from room temperature to about 1600° F. are acceptable for deforming the beta quenched metal depending upon the metal and amount of reduction taken in each rolling cycle. Annealing temperatures from about 40 1400° F. to about 1700° F. are acceptable, and the pre-

5  
10  
15  
20  
25  
30  
35

40  
45

6  
thickness. The temperature decreased during rolling to a finish temperature of 1650° F., and a majority of the rolling was carried out in the alpha-beta field. A test panel was cut from the hot band and heated at a temperature of 1950° F. for three minutes. The panel was then quenched by rapid immersion in a cold water bath. The beta quench produced an acicular type microstructure in the metal.

The beta quenched panel was then subjected to five 15% reduction rolling cycles at room temperature. The panel was line annealed for five minutes at 1600° F. followed by air cooling after each rolling cycle. The final anneal effected substantially complete recrystallization, and the finished cold rolled strip was free from internal cracking and showed no ridging when a 2-inch by 10-inch test piece was cold stretched to an elongation of about 10%. No ribbing was discernible either in the final product or at any stage after the beta quench. A specimen of the finished cold rolled strip was sectioned and polished and its microstructure found to be fine-grained and substantially completely recrystallized.

Another bar of Ti-5Al-2.5Sn alloy was unidirectionally hot rolled to 0.130 inch thickness from a temperature in the beta field with a majority of the reduction taking place in the alpha-beta field. A panel from the hot band was then heated at 1950° F. for five minutes and water quenched. The beta quenched panel was sandblasted and pickled and rolled at 1000° F. to effect a 60% reduction to 0.051 inch. The test piece was again sandblasted and pickled and was then annealed for ten minutes at 1650° F. and air cooled. No ribbing occurred during the rolling at 1000° F.; and, as indicated in Table A, the mechanical properties of the resulting strip were good. The microstructure was found to be completely recrystallized after the final anneal.

Three other panels from this hot band were processed in the same way and then subjected to one, two and three 20% reduction cold rolling cycles. Each cold rolling cycle was followed by an anneal at 1600° F. for a period of three to five minutes and air cooling. No ridging occurred when specimens were stretched to an elongation of at least 10%. The material did not rib during cold rolling, and good mechanical properties and low anisotropy were obtained as indicated in Table A. All bends in Table A and in the other tables appearing hereinafter were rated at 20× magnification with no observable rupture.

TABLE A

| Cold rolling          | Test gauge inch | Dir. | Ftu, K.s.i. | Fty, K.s.i. | Percent El <sup>*</sup> | E, p.s.i. × 10 <sup>6</sup> | 20X MBR R/T |
|-----------------------|-----------------|------|-------------|-------------|-------------------------|-----------------------------|-------------|
| None-----             | .051            | L    | 139.3       | 125.0       | 20.0                    | 16.3                        | 3.1         |
|                       |                 | T    | 134.3       | 128.2       | 21.0                    | 17.6                        | 3.1         |
| One 20% cycle-----    | .040            | L    | 134.1       | 118.4       | 20.0                    | 16.5                        | 3.8         |
|                       |                 | T    | 134.4       | 124.3       | 20.2                    | 17.2                        | 3.1         |
| Two 20% cycles-----   | .030            | L    | 134.8       | 122.1       | 17.0                    | 16.3                        | 3.0         |
|                       |                 | T    | 133.3       | 123.3       | 19.5                    | 17.7                        | 2.6         |
| Three 20% cycles----- | .024            | L    | 137.7       | 125.4       | 17.0                    | 16.9                        | 3.6         |
|                       |                 | T    | 136.2       | 123.7       | 19.2                    | 17.3                        | 2.7         |

\*One inch gauge.

cise temperature will be selected in accordance with the metal and the type of anneal utilized. The duration of the anneal will also vary with the metal being treated and the annealing temperature. Line anneals ranging from five to ten minutes have been used, and box anneals varying from sixteen to forty-eight hours have also been used.

The following non-limiting examples illustrate specific 65 embodiments of our process as applied to commercially pure titanium and to the representative titanium alloys, Ti-5Al-2.5Sn; Ti-6Al-4V and Ti-8Al-1Mo-1V.

#### EXAMPLE I

A sheet bar of an alloy containing 5% aluminum, 2.5% tin, balance titanium having a beta transus of 1900° F. ±25° was unidirectionally hot rolled from a temperature of about 2100° F. to produce a hot band of 0.135 inch 75

60  
65  
70  
75

The maximum acceptable bend radius for Ti-5Al-2.5Sn is 4.0 for .070 inch gauge and below and it is apparent that all specimens met this specification.

An additional bar of Ti-5Al-2.5Sn alloy was unidirectionally hot rolled to 0.149 inch thickness from a temperature in the beta field with the majority of the reduction taking place in the alpha-beta field. Two panels from the hot band were then heated at 1950° F. for five minutes and water quenched. Both beta quenched panels were then rolled to 0.057 inch, a total reduction of 60%. One panel was rolled at 1400° F. and the other at 1600° F. No ridging occurred during rolling and the microstructure of each panel showed complete recrystallization during rolling. Mechanical testing after line annealing for ten minutes at 1650° F. and air cooling showed low anisotropy, high tensile and bend ductility as indicated in Table B. No ridging occurred after 10% elongation.

TABLE B

| Rolling temp., ° F. | Dir. | Ftu<br>K.s.i. | Fty<br>K.s.i. | Percent<br>El* | E, p.s.i.<br>× 10 <sup>6</sup> | 20× |     |
|---------------------|------|---------------|---------------|----------------|--------------------------------|-----|-----|
|                     |      |               |               |                |                                | MBR | R/T |
| 1,400               | L    | 124.3         | 111.9         | 20.2           | 16.6                           | 3.5 |     |
|                     | T    | 120.9         | 114.1         | 18.7           | 17.3                           | 3.5 |     |
| 1,600               | L    | 122.6         | 111.4         | 22.2           | 16.6                           | 3.5 |     |
|                     | T    | 121.6         | 114.6         | 19.2           | 17.2                           | 3.5 |     |

\*One inch gauge.

## EXAMPLE II

A sheet bar of an alloy containing 6% aluminum, 4% vanadium, balance titanium having a beta transus of 1820° F. ±25° was unidirectionally hot rolled from a temperature of 1900° F. to produce a hot band of 0.140 inch thickness. The rolling finished at 1500° F.; and, therefore, a major portion of the reduction was accomplished in the alpha-beta field. A panel from the hot band was heated to a temperature of 1925° F. for five minutes and then rapidly quenched by immersion in water. The beta quench produced an acicular type microstructure in the metal.

The beta quenched panel was then cold rolled and annealed according to the following sequence:

Roll—15% reduction  
Anneal—7 minutes at 1500° F. AC  
Roll—15% reduction  
Anneal—7 minutes at 1500° F. AC  
Roll—15% reduction  
Anneal—48 hours at 1450° F. VC<sup>1</sup>  
Roll—20% reduction  
Anneal—6 minutes at 1600° F. AC

<sup>1</sup> Vacuum cool—30% slower than air cool.

The cold rolled panel was free from internal cracking and showed no ridging when a 3-inch by 10-inch test piece was stretched to an elongation of about 7%. No ribbing was discernible at any stage after the beta quench. A specimen of the finished cold rolled test piece was sectioned and polished and its microstructure found to be equiaxed fine-grained and substantially completely recrystallized.

A second bar of this alloy was unidirectionally hot rolled from a temperature in the beta field to thickness of 0.135 inch. A plurality of panels were cut from the hot band, and each panel was heated at 1950° F. for five minutes after which it was water quenched. Following the beta quench the panels were sandblasted and pickled in order to clean the surface of the metal. The panels were then rolled at 1000° F. to effect reductions of 15%, 20%, 25% and 30% after which each panel was further reduced 40% at 1000° F. A five minute anneal at 1650° F. and air cooling followed by sandblasting and pickling was used between reductions, and a final recrystallization anneal at 1450° F. for forty-eight hours with vacuum cooling was applied to each panel. The final panels exhibited good ductility and low anisotropy when tested. The test results are set forth in Table C. No ridging was observed during rolling subsequent to the beta quench, and no ridging occurred in the finished panels when elongated. The maximum acceptable bend radius for Ti-6Al-4V is 4.5 for 0.070 inch gauge and below and 5.0 for strip thicker than 0.070 inch. All specimens met these specifications.

A third bar of this alloy was unidirectionally hot rolled from a temperature in the beta field to a thickness of 0.175 inch. Two panels were cut from the hot band and heated for five minutes at 1950° F. followed by water quenching. The beta quenched panels were sandblasted and pickled to remove contamination. The panels were then rolled at 1400° F. and 1600° F. to 0.065 inch, a 60% reduction. Each panel was annealed at 1450° F. for forty-eight hours followed by vacuum cooling and pickling. The final microstructure of the panels was essentially completely recrystallized. Mechanical tests showed low anisotropy and good tensile and bend ductility as indicated in Table D. No ridging occurred on specimens pulled to 10% elongation.

10  
15

## TABLE D

| Rolling temp., ° F. | Dir. | Ftu<br>K.s.i. | Fty<br>K.s.i. | Percent<br>El* | E, p.s.i.<br>× 10 <sup>6</sup> | 20× |     |
|---------------------|------|---------------|---------------|----------------|--------------------------------|-----|-----|
|                     |      |               |               |                |                                | MBR | R/T |
| 1,400               | L    | 130.3         | 114.4         | 17.5           | 15.9                           | 3.5 |     |
|                     | T    | 127.0         | 120.0         | 18.0           | 16.8                           | 3.5 |     |
| 1,600               | L    | 130.7         | 113.6         | 19.0           | 15.9                           | 3.6 |     |
|                     | T    | 129.3         | 120.7         | 18.7           | 17.6                           | 3.7 |     |

\*One inch gauge.

## EXAMPLE III

25 A sheet bar of alloy containing 8% aluminum, 1% molybdenum, 1% vanadium, balance titanium having a beta transus of 1900° F. ±25° was unidirectionally hot rolled from a temperature of 2100° F. to produce a hot band of 0.120 inch thickness. The rolling finished at 1650° F., and the major portion thereof was carried out in the alpha-beta field as the bar cooled during rolling. A panel from the hot band was heated for five minutes at 1950° F. and quenched by immersion in water. The beta quench produced an acicular type microstructure in the metal.

30 The beta quenched panel was then subjected to cold rolling and annealing according to the following sequence:

Roll—10% reduction  
Anneal—48 hours at 1450° F. VC<sup>1</sup>  
Roll—15% reduction  
Anneal—7 minutes at 1500° F. AC  
Roll—15% reduction  
Anneal—7 minutes at 1500° F. AC  
Roll—15% reduction  
Anneal—48 hours at 1450° F. VC<sup>1</sup>  
Roll—15% reduction  
Anneal—6 minutes at 1650° F. AC

<sup>1</sup> Vacuum cool—30% slower than air cool.

35 40 45 50 The finished panel was free from internal cracking and showed no ridging when a 2-inch by 10-inch piece was cold stretched to an elongation of about 6%. No ribbing was discernible in the final product or at any stage during the processing of the panel after the beta quench. A specimen of the finished cold rolled panel was sectioned and polished and its microstructure found to be fine-grained and substantially completely recrystallized.

55 Another bar of Ti-8Al-1Mo-1V alloy was unidirectionally hot rolled from a temperature in the beta field to a hot band of 0.140 inch. Panels were cut from the hot band and annealed at 1950° F. for five minutes followed by quenching in water. Each beta quenched panel was

## TABLE C

| 1,000° F. cycles | Test gauge inch | Dir. | Ftu<br>K.s.i. | Fty<br>K.s.i. | Percent<br>El* | E,<br>p.s.i.<br>× 10 <sup>6</sup> |     | 20×<br>MBR<br>R/T |
|------------------|-----------------|------|---------------|---------------|----------------|-----------------------------------|-----|-------------------|
|                  |                 |      |               |               |                |                                   |     |                   |
| 15%-40%-----     | .075            | L    | 132.5         | 121.8         | 18.7           | 15.7                              | 3.3 |                   |
|                  |                 | T    | 133.5         | 123.9         | 18.5           | 17.6                              | 2.5 |                   |
| 20%-40%-----     | .071            | L    | 132.6         | 120.4         | 19.0           | 16.0                              | 3.5 |                   |
|                  |                 | T    | 132.6         | 125.1         | 19.5           | 18.1                              | 3.5 |                   |
| 25%-40%-----     | .066            | L    | 134.5         | 121.2         | 18.5           | 15.8                              | 3.8 |                   |
|                  |                 | T    | 133.5         | 125.4         | 19.0           | 17.7                              | 3.0 |                   |
| 30%-40%-----     | .060            | L    | 132.4         | 119.9         | 19.3           | 15.9                              | 3.9 |                   |
|                  |                 | T    | 130.7         | 121.5         | 18.3           | 17.7                              | 3.5 |                   |

\*One inch gauge.

then sandblasted and pickled and rolled at 1000° F. to effect a 30% reduction, annealed at 1650° F. for five minutes followed by air cooling, rolled at 1000° F. to effect a 40% reduction, sandblasted and pickled and annealed for forty-eight hours at 1450° F. followed by vacuum cooling. The microstructure of the panels was fine grained and substantially completely recrystallized after the forty-eight hour anneal. Individual panels were then cold rolled through one, two, three and four 20% reduction cycles with a five minute anneal at 1650° F. followed by air cooling between each cycle. Subsequent to the last rolling cycle, each panel was annealed at 1450° F. for forty-eight hours followed by vacuum cooling to effect a second recrystallization. Each of the panels was successfully cold rolled without internal shear cracking. As shown in Table E, the metal was ductile and anisotropy was low. No ribbing was observed during rolling and specimens were elongated without ridging. The acceptable bend radius for Ti-8Al-1Mo-1V is 4.0 for 0.070 inch gauge and below and all samples tested met this specification.

TABLE G

| Rolling temp., ° F. | Dir. | Ftu    | Fty    | Percent | E, p.s.i.         | 20X     |
|---------------------|------|--------|--------|---------|-------------------|---------|
|                     |      | K.s.i. | K.s.i. | El*     | × 10 <sup>6</sup> | MBR R/T |
| 5,1400-----         | L    | 138.1  | 128.6  | 20.7    | 16.9              | 3.8     |
|                     | T    | 132.5  | 127.5  | 20.5    | 18.1              | 3.7     |
| 5,1600-----         | L    | 140.6  | 128.3  | 21.2    | 17.1              | 4.0     |
|                     | T    | 135.0  | 127.5  | 20.2    | 17.9              | 3.7     |

\*One inch gauge.

## EXAMPLE IV

A panel of commercially pure titanium, Ti-75A, was cut from a unidirectionally hot rolled band having a thickness of .150 inch containing 0.304% oxygen and having a beta transus of 1725-1750° F. The panel was cold rolled to 0.10 inch and was heated at a temperature of 1800° F. for 2.5 minutes. The panel was then quenched by rapid immersion in a cold water bath. The beta quench produced an acicular type microstructure in the metal. The beta quenched panel was then subjected to four cycles of 15% reduction at room temperature using

TABLE E

| Cold rolling          | Test gauge, inch | Dir. | Ftu, K.s.i. | Fty, K.s.i. | Percent El* | E, p.s.i. × 10 <sup>6</sup> | 20X MBR R/T |
|-----------------------|------------------|------|-------------|-------------|-------------|-----------------------------|-------------|
| None-----             | .055             | L    | 138.6       | 129.5       | 20.0        | 16.9                        | 3.7         |
|                       |                  | T    | 134.5       | 127.5       | 22.0        | 17.9                        | 2.9         |
| One 20% cycle-----    | .044             | L    | 137.9       | 127.4       | 20.0        | 16.8                        | 3.9         |
|                       |                  | T    | 135.0       | 124.7       | 19.5        | 18.0                        | 3.5         |
| Two 20% cycles-----   | .033             | L    | 134.6       | 122.6       | 19.5        | 16.7                        | 3.7         |
|                       |                  | T    | 129.0       | 120.4       | 21.0        | 17.7                        | 3.1         |
| Three 20% cycles----- | .024             | L    | 131.8       | 122.3       | 21.8        | 18.2                        | N.T.        |
|                       |                  | T    | 126.9       | 121.5       | 21.5        | 18.4                        | 3.2         |
| Four 20% cycles-----  | .018             | L    | 131.8       | 118.5       | 20.5        | 15.7                        | 3.9         |
|                       |                  | T    | 127.3       | 118.5       | 23.8        | 17.2                        | 3.2         |

\*One inch gauge.  
N.T.—Tot tested.

A pair of Ti-8Al-1Mo-1V alloy panels were treated in the same way as the panels in the immediately preceding group except that after the first 30% reduction at 1000° F. and the following anneal, the panels were rerolled at 1000° F. through two and three 30% reduction cycles at 1000° F. Each rolling cycle was followed by a five minute anneal at 1650° F. and air cooling, and the last rolling cycle was followed by sandblasting, pickling and a forty-eight hour recrystallization anneal at 1450° F. and vacuum cooling. These panels also exhibited substantially complete recrystallization and directionality was low as shown in Table F. No ribbing occurred during rolling and the panels were elongated without ridging.

40 1400° F. seven minute intermediate anneals. The final anneal effected substantially complete recrystallization, and the finished cold rolled strip was free from internal cracking and showed no ridging when a 2-inch by 10-inch test piece was cold stretched to an elongation of about 10%. No ribbing was discernible either in the final product or at any stage after the beta quench. A specimen of the finished cold rolled strip was sectioned and polished and its microstructure found to be recrystallized.

45 Six additional panels from the same 0.150 inch hot band were heated at 1850° F. for five minutes and then rapidly cooled by immersion in water. The beta quenched panels were sandblasted and pickled and rolled a total of 50 60% at 600° F., 800° F., 1000° F., 1200° F., 1400° F.

TABLE F

| 1,000° F. cycles | Test gauge, inch | Dir. | Ftu, K.s.i. | Fty, K.s.i. | Percent El* | E, p.s.i. × 10 <sup>6</sup> | 20X MBR R/T |
|------------------|------------------|------|-------------|-------------|-------------|-----------------------------|-------------|
| Three 30%-----   | .047             | L    | 138.6       | 128.4       | 19.7        | 16.9                        | 3.6         |
|                  |                  | T    | 134.1       | 129.0       | 21.2        | 17.7                        | 3.6         |
| Four 30%-----    | .029             | L    | 134.5       | 125.7       | 18.5        | 17.0                        | 3.5         |
|                  |                  | T    | 129.5       | 126.3       | 18.5        | 17.1                        | 3.9         |

\*One inch gauge.

Two additional Ti-8Al-1Mo-1V panels from the same unidirectionally hot rolled bar were heated at 1950° F. for five minutes and water quenched. The beta quenched panels were then rolled to 0.053 inch, a 60% reduction, at 1400° F. and 1600° F. The panels were descaled and pickled and box annealed at 1450° F. for forty-eight hours followed by vacuum cooling and pickling. The resulting microstructure of each panel was essentially completely recrystallized. As indicated in Table G, mechanical testing showed low anisotropy and high tensile and bend ductility. No ridging occurred on specimens pulled at 10% elongation.

65 and 1600° F. respectively. The panels rolled at 1000° F. and below were completely recrystallized into equiaxed grains by a 1650° F. ten minute anneal followed by air cooling. The tests performed on these panels showed no ridging, low anisotropy and high tensile and bend ductility as shown in Table H. All specimens met the bend 70 specifications of 2.5 for 0.060 inch and below and 3.0 for strip thicker than 0.060 inch. The panels rolled at 1200° F. and above recrystallized simultaneously with rolling. These panels demonstrated good mechanical properties and high ductility without an anneal. A 1650° F. ten minute anneal followed by air cooling further 75

increased the ductility by completely stress relieving the hot rolled structure.

60% at 1000° F. and annealed for ten minutes at 1650° F. followed by air cooling in an attempt to recrystallize

TABLE H

| Rolling temp., ° F. | Test gauge, inch | Dir. | Ftu K.s.i. | Fty K.s.i. | Percent El <sup>1</sup> * | E, p.s.i. × 10 <sup>6</sup> | 20X MBR RT |
|---------------------|------------------|------|------------|------------|---------------------------|-----------------------------|------------|
| 600.....            | .054             | L    | 97.1       | 72.8       | 31.0                      | 14.9                        | 2.1        |
|                     |                  | T    | 96.2       | 80.1       | 29.0                      | 17.3                        | 2.0        |
| 800.....            | .059             | L    | 94.2       | 66.5       | 33.0                      | 15.5                        | 2.0        |
|                     |                  | T    | 96.1       | 80.9       | 30.5                      | 16.9                        | 2.1        |
| 1,000.....          | .055             | L    | 96.4       | 73.0       | 28.0                      | 15.4                        | 2.1        |
|                     |                  | T    | 93.0       | 77.5       | 28.5                      | 16.6                        | 2.1        |
| 1,200.....          | .055             | L    | 96.0       | 70.4       | 32.0                      | 15.6                        | 2.1        |
|                     |                  | T    | 104.7      | 82.0       | 29.0                      | 19.5                        | 2.1        |
| 1,400.....          | .054             | L    | 97.5       | 71.4       | 33.0                      | 15.7                        | 2.1        |
|                     |                  | T    | 96.9       | 78.8       | 28.5                      | 17.0                        | 2.1        |
| 1,600.....          | .055             | L    | 94.6       | 64.5       | 36.0                      | 15.1                        | 2.1        |
|                     |                  | T    | 100.0      | 81.8       | 29.0                      | 17.4                        | 2.1        |

\*One inch gauge.

The effect of the beta quench on the ribbing and ridging characteristics of titanium alloy is clearly shown by the results of a test in which hot band panels of Ti-5Al-2.5Sn alloy were rolled at 1000° F. to effect a 60% reduction and box annealed at 1450° F. for forty-eight hours followed by vacuum cooling. One panel had been beta quenched prior to rolling and annealing and the second panel was rolled as received. The microstructures of both panels were recrystallized to the same extent. However, when the panel which was not beta quenched was pulled to 10% elongation, ridging occurred while no ridging took place in the beta quenched panel.

Panels of Ti-8Al-1Mo-1V alloy and Ti-6Al-4V alloy were also cold rolled from non-beta quenched hot bands, and in each instance ridging occurred when the rolled panels were stretched at less than 10% elongation.

In order to ascertain the necessity of rapid cooling from the beta field to create the acicular type microstructure, comparative tests were conducted. The tests and the results are set forth hereinafter.

#### Test A

The test panels of Ti-8Al-1Mo-1V alloy were taken from a unidirectionally hot rolled hot band at 0.150 inch gauge and were heated at a temperature of 1950° F. for five minutes. One of the panels was water quenched below the beta transus, and the other was air cooled. Metallographic examination showed that the quenched panel had an acicular alpha structure, whereas the air cooled panel had a lamellar alpha structure. Both panels were then rolled at 1000° F. to effect a 30% reduction, annealed at 1650° F. for five minutes followed by air cooling and rolled again at 1000° F. to effect a 40% reduction. Both panels were then box annealed at 1450° F. for forty-eight hours followed by vacuum cooling. Examination of the panels showed that the micro-structure of the air cooled panel was not completely recrystallized and still showed remnants of the beta heated structure while substantially complete recrystallization occurred in the quenched panel. In order to determine the cold rollability of the metal, both panels were cold rolled through three cycles of 15% reduction with a five minute line anneal at 1650° F. with air cooling after each reduction. Internal shear cracking occurred in the air cooled panel during the first cold reduction, and the cracking increased during the second and third reductions. No cracks occurred in the panel subjected to the beta quench even after the third cycle of 15% reduction.

#### Test B

Two panels of Ti-5Al-2.5Sn alloy were taken from a hot band at 0.130 gauge and heated at 1950° F. for five minutes. One of the panels was air cooled to below the beta transus and the other was water quenched. Metallographic examination of the panels showed an acicular alpha structure in the quenched panel and a lamellar alpha structure in the air cooled panel. Both panels were then reduced

20 the microstructure. The microstructure of the air cooled panel was not completely recrystallized, whereas that of the quenched panel was. The panels were then cold rolled through three cycles of 15%, 20% and 25% reduction, and serious cracking occurred in the slowly cooled panel during the 15% reduction cycle and the cracking increased during the next two cycles. No cracking occurred in the panel subjected to the beta quench.

25 The results of tests A and B clearly show that cooling to a temperature below the beta transus at a rate sufficiently rapid to create an acicular alpha structure prevents internal shear cracking and is essential to obtain complete recrystallization.

30 As will be appreciated by those skilled in the art, the degree of reduction must be considered in conjunction with the rolling temperature and the desired final gauge in order to produce recrystallized strip having good ductility and minimum anisotropy. For example, Ti-8Al-1Mo-1V alloy can be recrystallized by two 20% reductions and a 30% reduction at 600° F. with intermediate five minute anneals at 1600° F. followed by a final recrystallization anneal at 1450° F. for forty-eight hours or by a single 35 60% reduction at 1200° F. followed by a 1450° F. anneal for forty-eight hours.

35 A temperature which has proved advantageous for rolling Ti-5Al-2.5Sn, Ti-6Al-4V and Ti-8Al-1Mo-1V alloys is 1000° F. The Ti-5Al-2.5Sn can be directly reduced 60% at this temperature without any intermediate stress relief anneal as is shown in Example I. The Ti-6Al-4V and Ti-8Al-1Mo-1V alloys must be reduced in at least two cycles at 1000° F. with an intermediate partial stress relief anneal. The initial reduction for Ti-6Al-4V may vary from about 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 86

quench the hot band directly with no preliminary rolling so that a recrystallized strip of reasonable thickness may be obtained for subsequent cold finishing.

After recrystallizing by rolling at elevated temperatures and annealing, the titanium strip alloys can be cold rolled without internally shear cracking up to 100% more than is possible by directly cold rolling beta quenched material. Subsequent to recrystallization they can also be cold rolled through several cycles of reduction with intermediate anneals down to very thin gauge. The proper anneal after cold rolling will result in a second complete recrystallization. For example, a fifteen minute anneal at 1650° F. will recrystallize Ti-5A1-2.5 Sn alloy for the second time after it has been cold-rolled through one or more 20% reductions; and a forty-eight hour anneal at 1450° F. followed by vacuum cooling will recrystallize Ti-8A1-1Mo-1V and Ti-6A1-4V alloys for the second time after they have been cold rolled through one or more 20% reductions.

Tests have shown that when rolling at room temperature and annealing are used to effect recrystallization, the maximum reduction possible per cycle without internal shear cracking of the beta quenched hot band is about 10 to 15% for the Ti-6A1-4V and Ti-8A1-1Mo-1V alloys and about 15 to 20% for Ti-5A1-2.5 Sn alloy. 25 Heavier cold reductions than these after the beta quench cause internal shear cracking of the metal. However, it is possible to obtain a finished strip with a recrystallized microstructure by effecting larger cold reductions prior to the beta quench and rolling to gauge in one or 30 two cycles after the beta quench depending upon the alloy. As pointed out heretofore, it is not necessary that the metal be beta quenched immediately after unidirectionally hot rolling to hot band so long as sufficient reduction is effected after the beta quench to impart strain to the metal so that substantially complete recrystallization will occur during the final anneal. The desired finish gauge is, therefore, a determining factor in respect of the degree of reduction taken after the beta quench and the reduction temperature, as the metal must be reduced by an amount sufficient to create the required strain 35 after the beta quench. The temperature of rolling will determine the degree of reduction required to impart strain to the metal as less reduction is required at lower temperatures to create the strain necessary for subsequent recrystallization.

The recrystallization anneal provides the driving energy necessary to recrystallize the strained microstructures into strain free equiaxed grains; therefore, the exact temperatures and times used are dependent on the rolling cycles used. The recrystallization temperature selected must not be above the beta transus since the object is to recrystallize the alpha structure and not transform alpha into beta. For alpha type titanium alloys a relatively short time line anneal will result in complete recrystallization. For example, a ten minute anneal at 1650° F. followed by air cooling is satisfactory for Ti-5A1-2.5 Sn. Much longer anneals are required for the alpha-beta type alloys and Ti-8A1-1Mo-1V and Ti-6A1-4V require forty-eight hour anneals at 1450° F. for effecting substantially complete recrystallization. The longer anneals are termed box anneals and are performed on coils generally in a vacuum furnace to prevent contamination of the metal surface, although the use of a vacuum furnace is not a requirement for our process. Temperatures for vacuum anneals are limited to about 1450° F. because at higher temperatures titanium tends to stick together when under a vacuum; and such is, of course, detrimental to coil annealing.

It should be understood that descaling and pickling of the strip is not a requirement of our process. Descaling and pickling clean the surface and reduce further contamination, and removal of oxides and scale prior to a rolling pass prevents enlarging and spreading these defects.

The method of our invention is advantageous in the

production of elongated strip titanium and certain titanium base alloys from unidirectionally hot rolled hot band. The strip produced by our method is completely free from ribbing, has no tendency toward ridging and has minimum anisotropy. The beta quench and subsequent deformation and annealing provide equiaxed recrystallized grain structure, and the material can readily be finish cold rolled without internal cracking. Additionally, the material has good ductility and can, therefore, meet bend specifications.

10 While preferred embodiments of the invention have been described, it may be otherwise embodied within the scope of the appended claims.

We claim:

- 15 1. A method for producing strip of a metal selected from the group consisting of commercially pure titanium, alpha stabilized alpha type titanium base alloys and alpha stabilized alpha-beta type titanium base alloys, which comprises:
  - (1) unidirectionally hot rolling a body of said metal to reduce said body to an elongated hot band, said rolling being initiated at a temperature requiring a substantial amount of said reduction to occur in the alpha-beta field of said metal,
  - (2) heating said hot band at a temperature above the beta transus of said metal to completely transform the crystal structure of said metal to the beta phase,
  - (3) rapidly cooling said hot band from said temperature above the beta transus of said metal to a temperature below said beta transus to produce an acicular type microstructure in the metal and
  - (4) subjecting said rapidly cooled hot band to the steps of rolling and annealing at temperatures below said beta transus to produce an elongated strip having a substantially completely recrystallized microstructure.
- 20 2. A method as set forth in claim 1 including rolling said hot band prior to heating said hot band at a temperature above said beta transus of said metal to effect a reduction in the thickness of said hot band prior to said heating.
- 35 3. A method as set forth in claim 1 including stress relief annealing said rapidly cooled hot band at a temperature below the beta transus of said metal prior to rolling said hot band.
- 40 4. A method as set forth in claim 1 including unidirectional hot rolling of said body is initiated at a temperature above the beta transus of said metal.
- 45 5. A method as set forth in claim 1 wherein said unidirectional hot rolling of said body is initiated at a temperature sufficiently high in the alpha-beta field of said metal that the beta phase of said metal is unstable.
- 50 6. A method as set forth in claim 1 wherein said heating of said hot band is at a temperature between the beta transus of said metal and about 150° F. above the beta transus of said metal.
- 55 7. A method as set forth in claim 1 wherein said heated hot band is rapidly cooled from said temperature above the beta transus of said metal by immersion.
- 60 8. A method as set forth in claim 1 wherein said heated hot band is rapidly cooled from said temperature above the beta transus of said metal to room temperature.
- 65 9. A method as set forth in claim 1 wherein said rolling of said rapidly cooled hot band is at a temperature between room temperature and about 1600° F.
- 70 10. A method as set forth in claim 1 wherein said rolling of said rapidly cooled hot band is at about 1000° F.
- 75 11. A method as set forth in claim 1 wherein said rolling of said rapidly cooled hot band consists of a plurality of rolling cycles between room temperature and about 300° F. and wherein said annealing consists of an anneal after each rolling cycle.
12. A method as set forth in claim 11 including rolling said hot band between room temperature and about 300° F. to effect a substantial reduction prior to heating

said hot band at a temperature above the beta transus of said metal.

13. A method as set forth in claim 1 wherein said metal is an alloy consisting essentially of 5% aluminum, 2.5% tin, balance titanium, and wherein said rolling of said rapidly cooled hot band consists of a plurality of cycles at room temperature with a maximum reduction of 15% to 20% in each cycle and said annealing consists of heating at about 1600° F. for about five minutes after each rolling cycle whereby the final anneal produces said substantially completely recrystallized microstructure in said elongated strip.

14. A method as set forth in claim 1 wherein said metal is an alloy consisting essentially of 5% aluminum, 2.5% tin, balance titanium, and wherein said rolling of said rapidly cooled hot band consists of a single cycle at about 1000° F. to effect a reduction of about 60% and said annealing consists of heating at about 1650° F. for about ten minutes to produce said substantially completely recrystallized microstructure in said elongated strip.

15. A method as set forth in claim 1 wherein said metal is an alloy consisting essentially of 8% aluminum, 1% molybdenum, 1% vanadium, balance titanium, and wherein said rolling of said rapidly cooled hot band consists of a plurality of cycles at room temperature with a maximum reduction of 10% to 15% in each cycle and said annealing consists of heating after each rolling cycle, the final heating being at about 1450° F. for about forty-eight hours to produce said substantially completely recrystallized microstructure in said elongated strip.

16. A method as set forth in claim 1 wherein said metal is an alloy consisting essentially of 8% aluminum, 1% vanadium, balance titanium, and wherein said rolling of said rapidly cooled hot band consists of a plurality of cycles at about 1000° F. with a reduction of 20% to 35% in each cycle and said annealing consists of heating at about 1650° F. for above five minutes between rolling cycles and heating at about 1450° F. for about forty-eight hours after the final rolling cycle to produce said substantially recrystallized microstructure in said elongated strip.

17. A method as set forth in claim 1 wherein said metal is an alloy consisting essentially of 8% aluminum, 1% molybdenum, 1% vanadium, balance titanium, and wherein said rolling of said rapidly cooled hot band consists of a first cycle at about 1000° F. to effect a reduction of about 30% and a second cycle at about 1000° F. to effect a further reduction of about 40% and said annealing consists of heating at about 1650° F. for above five minutes after said first cycle and heating at about 1450° F. for about forty-eight hours after said second cycle to produce said substantially completely recrystallized microstructure in said elongated strip.

18. A method as set forth in claim 1 wherein said metal is an alloy consisting essentially of 6% aluminum, 4% vanadium, balance titanium, and wherein said rolling of said rapidly cooled hot band consists of a plurality of cycles at room temperature to effect a maximum reduction of 10% to 15% in each cycle and said annealing consists of heating after each rolling cycle, the final heating being at about 1450° F. for about forty-eight hours to produce said substantially completely recrystallized microstructure in said elongated strip.

19. A method as set forth in claim 1 wherein said metal is an alloy consisting essentially of 6% aluminum, 4% vanadium, balance titanium, and wherein said rolling of said rapidly cooled hot band consists of a plurality of cycles at about 1000° F. to effect a reduction of 15% to 35% in each cycle and said annealing consists of heating at about 1650° F. for five minutes between rolling cycles and heating at about 1450° F. for about forty-eight hours

after the final rolling cycle to produce said substantially completely recrystallized microstructure in said elongated strip.

5 20. A method as set forth in claim 1 wherein said metal is an alloy consisting essentially of 6% aluminum, 4% vanadium, balance titanium, and wherein said rolling of said rapidly cooled hot band consists of a first cycle at about 1000° F. to effect a reduction of about 25% and a second cycle at about 1000° F. to effect a reduction of about 40% and said annealing consists of heating at about 1650° F. for about five minutes after said first cycle and heating at about 1450° F. for about forty-eight hours after said second cycle to produce said substantially completely recrystallized microstructure in said elongated strip.

10 21. A method as set forth in claim 1 wherein said metal is commercially pure titanium, and wherein said rolling of said rapidly cooled hot band consists of a plurality of cycles at room temperature with a reduction of 15% in each cycle and said annealing consists of heating at about 1400° F. for about seven minutes after each rolling cycle whereby the final anneal produces said substantially completely recrystallized microstructure in said elongated strip.

15 22. A method as set forth in claim 1 wherein said metal is commercially pure titanium, and wherein said rolling of said rapidly cooled hot band consists of a single cycle at about 1000° F. to effect a reduction of about 60% and said annealing consists of heating at about 1650° F. for about ten minutes to produce said substantially completely recrystallized microstructure in said elongated strip.

20 23. A method for producing strip of a metal selected from the group consisting of commercially pure titanium and a titanium alloy consisting essentially of 5% aluminum, 2.5% tin, balance titanium, which comprises:

25 (1) unidirectionally hot rolling a body of said metal to reduce said body to an elongated hot band, said rolling being initiated at a temperature requiring a substantial amount of said reduction to occur in the alpha-beta field of said metal,

(2) heating said hot band at a temperature above the beta transus of said metal to completely transform the crystal structure of said metal to the beta phase,

(3) rapidly cooling said hot band from said temperature above the beta transus of said metal to a temperature below said beta transus to produce an acicular type microstructure in the metal and

(4) rolling said rapidly cooled hot band at a temperature below the beta transus of said metal and sufficiently high to cause recrystallization of the microstructure during said rolling, whereby said rolling produces an elongated strip having a substantially completely recrystallized microstructure.

24. A method as set forth in claim 23 wherein said metal is an alloy consisting essentially of 5% aluminum, 2.5% tin, balance titanium, and wherein said rolling of said rapidly cooled hot band is at a temperature between about 1200° F. and 1400° F.

25 25. A method as set forth in claim 23 wherein said metal is commercially pure titanium, and wherein said rolling of said rapidly cooled hot band is at a temperature between about 1000° F. and 1200° F.

#### References Cited

#### UNITED STATES PATENTS

3,394,036 7/1968 Parris ----- 148—11.5  
3,169,085 2/1965 Newman ----- 148—11.5

L. DEWAYNE RUTLEDGE, Primary Examiner

W. W. STALLARD, Assistant Examiner

UNITED STATES PATENT OFFICE  
CERTIFICATE OF CORRECTION

Patent No. 3,492,172

January 27, 1970

Adrian Burt Sauvageot et al.

It is certified that error appears in the above identified patent and that said Letters Patent are hereby corrected as shown below:

Column 3, line 51, "heat" should read -- near --. Column 5, line 40, "rolling annealing" should read -- rolling and annealing --. Column 9, at the bottom of Table E, "Tot tested." should read -- Not tested. --. Column 11, in the last heading in Table H, "RT" should read -- R/T --; same column 11, line 41 "The" should read -- Two --. Column 14, line 25, "heaing" should read -- heating --. Column 15, line 32, "1% molybdenum," should be inserted after "aluminum,".

Signed and sealed this 23rd day of June 1970.

(SEAL)

Attest:

EDWARD M. FLETCHER, JR.  
Attesting Officer

WILLIAM E. SCHUYLER, JR.  
Commissioner of Patents